

## 1

3,087,775

## PRODUCTION OF ALKALI-SOLUBLE CELLULOSIC TEXTILE MATERIALS BY THE NITRIC ACID TREATMENT OF PARTIALLY ETHERIFIED COTTONS

Robert M. Reinhardt and Terrence W. Fenner, New Orleans, La., assignors to the United States of America as represented by the Secretary of Agriculture

No Drawing. Filed June 1, 1960, Ser. No. 33,350

8 Claims. (Cl. 8—116)

(Granted under Title 35, U.S. Code (1952), sec. 266)

A non-exclusive, irrevocable royalty-free license in the invention herein described, throughout the world for all purposes of the United States Government, with the power to grant sublicenses for such purposes, is hereby granted to the Government of the United States of America.

This invention relates to alkali-soluble cellulosic textile materials and methods of their production.

It is known that certain chemical modifications of cotton can be employed to prepare cellulosic derivatives which are alkali-soluble. However, many of those chemical modifications involve the use of the uneconomical reagents and/or uneconomical conditions of reaction. Further, many of these chemical modifications results in non-fibrous products or products which are so weakened and degraded that their value as textile materials is lost.

To be a useful article of commerce for textile usage, an alkali-soluble cellulosic textile material must possess enough strength to withstand the rigorous stresses and strains of processing on normal textile machinery. Along with these substantial strength requirements, because of the transient uses for which these textile materials are employed, their solubility must be sufficient to allow essentially complete removal of these textile members without undue complications to normal plant practices.

It is an object of this invention to provide a process for the production of alkali-soluble cellulosic textile materials which possess the strength and solubility characteristics necessary for industrial utilization. This objective is accomplished by a two step treatment: first, cotton textile materials are partially etherified to a low degree of substitution (D.S., the average number of substituent ether groups per anhydroglucose unit), in the range of from about 0.01 to about 0.6, and secondly, treatment of the partially etherified cotton with aqueous solutions of nitric acid. The process may be carried out on fabric, thread, yarn, or fiber.

It is a further objective of this invention to provide a process which is more economical than conventional processes in that only inexpensive reagents are used and in that more economical reaction conditions, notably shorter reaction times, lower reaction temperatures, and more dilute concentrations of reagent may be employed in the nitric acid treatment step than would be operative without the unique complementary effect of the combined steps of the two step process.

As is known to those skilled in the art, nitric acid treatments of cellulose have been used to prepare alkali-soluble materials. In the prior art, however, the products have been either highly nitrated materials (nitrocellulose) prepared under rigorous, usually anhydrous, reaction conditions with nitric acid and strong dehydrating agents, or materials nitrated to a lower degree but under conditions requiring mixed reagent techniques such as the use of nitric acid-phosphoric acid or nitric acid-sulfuric acid solutions, or materials which are not textile fibers but are produced in solution or are cast as films.

In the present invention the nitric acid treatment is carried out on partially etherified cottons. It is not necessary to use anhydrous conditions, dehydrating compounds

## 2

or mixed acid techniques. A fibrous product is produced which has good strength and is soluble in alkaline solutions. Further, by using partially etherified cottons instead of native or mercerized cotton as a starting material, less drastic conditions may be employed in nitric acid treatment step. With partially etherified cottons, products with higher solubility are obtained with more dilute concentrations of nitric acid, shorter treatment times, and lower temperatures than if the nitric acid treatment was carried out on native or mercerized cotton.

The two step treatment accomplishes the objectives through multiple effects. In the first or partial etherification step, a small amount of ether groups are introduced. These ether groups are alkali-solubilizing and would result in an alkali-soluble material if the etherification was carried out to greater extent. Further, these ether groups exert a swelling effect which makes the partially etherified cotton highly accessible for reaction in the nitric acid treatment step.

The preferred partially etherified cottons which may be employed in the process of this invention include partially aminoethylated, carbamoylethylated, carboxyethylated, carboxymethylated, cyanoethylated, hydroxyethylated, and phosphonomethylated cotton.

In the second or nitric acid treatment step, three chemical reactions may take place: nitration of cellulosic hydroxyls, oxidation along the cellulosic chain, and hydrolysis of glucosidic linkages of the cellulosic chain. All three reactions are efficacious in producing alkali solubility.

In the nitric acid treatment step, nitration of the cellulosic hydroxyls proceeds only to a low degree as evidenced by a modified Kjeldahl nitrogen analysis of the products. The nitrogen introduced is usually 1.2% or less. The low extent of oxidation during this step may be estimated by carboxyl and carbonyl analysis. Although some hydrolytic cleavage of glucosidic linkages takes place, this cleavage is not extensive as evidenced by the considerable strength retained by the product. Drastic loss of strength is a consequence of a relatively small amount of cleavage of glucosidic linkages. The extent of this cleavage may be more accurately estimated by D.P. (degree of polymerization) determinations.

No claim is made singly for the partial etherification or for the nitric acid treatment step. The process of this invention utilizes the unique complementary or synergistic effect of the combination of the two treatments.

The partial etherification step may be carried out by any of the known methods which will be apparent to those skilled in the art.

Partial aminoethylation of cotton may be carried out, for example, as described by Guthrie in Textile Research Journal 17, 625-9 (1957). The aminoethyl ether of cellulose may be represented by the formula



in which R represents the anhydroglucose unit.

Partial carbamoylation of cotton may be carried out, for example, as described by Frick, Reeves, and Guthrie in Textile Research Journal 27, 294-9 (1957). The carbamoyl ether of cellulose may be represented by the formula  $\text{ROCH}_2\text{CH}_2\text{C}(\text{O})\text{NH}_2$  in which R represents the anhydroglucose unit.

Partial carboxylation of cotton may be carried out, for example, as described by Daul, Reinhardt, and Reid in Textile Research Journal 25, 246-53 (1955). The carboxyethyl ether of cellulose may be represented by the formula  $\text{ROCH}_2\text{CH}_2\text{COOH}$  in which R represents the anhydroglucose unit.

Partial carboxymethylation of cotton may be carried out, for example, as described by Daul, Reinhardt, and Reid in Textile Research Journal 22, 787-92 (1952). The

carboxymethyl ether of cellulose may be represented by the formula  $\text{ROCH}_2\text{COOH}$  in which R represents the anhydroglucose unit.

Partial cyanoethylation of cotton may be carried out, for example, as described by Daul, Reinhardt, and Reid in Textile Research Journal 25, 246-53 (1955). The cyanoethyl ether of cellulose may be represented by the formula  $\text{ROCH}_2\text{CH}_2\text{CN}$  in which R represents the anhydroglucose unit.

Partial hydroxyethylation of cotton may be carried out, for example, as described by Lawrie, Reynolds, and Ward in Journal of the Society of Dyers and Colourists 56, 6-17 (1940). The hydroxyethyl ether of cellulose may be represented by the formula  $\text{ROCH}_2\text{CH}_2\text{OH}$  in which R represents the anhydroglucose unit.

Partial phosphonomethylation of cotton may be carried out, for example, as described by Drake, Reeves, and Guthrie in Textile Research Journal 29, 270-5 (1959). The phosphonomethyl ether of cellulose may be represented by the formula  $\text{ROCH}_2\text{P}(\text{O})(\text{OH})_2$  in which R represents the anhydroglucose unit.

Partially etherified cottons with a degree of substitution of from about 0.04 to about 0.55 are preferred for the process of this invention. The degree of substitution and the severity of conditions required in the nitric acid treatment for good alkali-solubility are inversely related.

In the present invention, the nitric acid treatment step may be carried out within widely varying limits. The treatment may be effected at temperatures ranging from about room temperature to boiling and at nitric acid concentrations varying from about 10% to about 70%. With higher temperatures, the treatment time is reduced and may be as little as a few seconds. The treatment temperature is correspondingly adjusted in inverse relation to treatment time. With the lower concentrations of nitric acid the time of treatment required is extended and may range to periods of 24 hours or longer. For the lower concentrations of nitric acid, the time of treatment necessary may thus be reduced by an adjustment towards higher temperatures.

The preferred range of conditions for the nitric acid treatment step thus encompasses treatment times of from about 0.5 minute to about 75 minutes, at temperatures of from about room temperature to the boiling temperature of the nitric acid solution, using concentrations of nitric acid of about 10% to about 70%, the time and temperature of the nitric acid treatment being inversely related to the nitric acid concentration.

Uses for alkali-soluble textile material are well known in the art. Among such uses are the preparation of open work fabrics by weaving soluble yarns and ordinary yarns in such a manner that upon dissolution of the soluble yarns the open-work pattern effect is produced in the fabric. Other uses may include utilization of alkali-soluble threads for basting or for connecting threads in the string-sock knitting process. The soluble members are readily removed by a subsequent alkali treatment. Alkali-soluble fabric is used as a backing cloth in a process for the manufacture of lace.

Having thus described in a general way the operation of the process of this invention, details of the process are listed below in specific examples which illustrate the application of the process to cotton textile materials.

The following laboratory techniques were used for determination of strength and alkali-solubility of the products.

*Determination of strength.*—The strength of the cellulosic textile materials was determined on one-inch strips by the standard test method of the American Society for Testing Materials as specified by A.S.T.M. Committee D-13 in "Standard General Methods of Testing Woven Textile Fabrics," Philadelphia, Pennsylvania, 1951, test method D39-49. The results are expressed as the percentage of the original strength of the fabric which is retained after the treatment.

*Determination of alkali-solubility.*—Approximately one gram of air-equilibrated cellulose textile material was accurately weighed on an analytical balance. The sample was transferred to a flask containing a boiling 10% aqueous solution of sodium hydroxide in an amount sufficient to give a 100:1 liquor to sample ratio, by weight. The solution containing the sample was maintained at boiling for 10 minutes. At the end of this period, the solution and residue were quantitatively transferred to a previously weighed centrifuge tube. The tube was then centrifuged for 8 minutes at 1700 r.p.m. to affect separation of the residue and clear supernatant solution. The solution was decanted and the residue washed twice with distilled water, twice with dilute acetic acid solution, and then four times with distilled water. The residue was then dried, equilibrated, and weighed in the analytical balance. From the weight of the residue, the alkali-solubility of the sample was calculated:

$$\text{Percent alkali-solubility} = 100 - \left[ \frac{\text{Wt. of Residue}}{\text{Wt. of Sample}} \times 100 \right]$$

#### EXAMPLE 1

Samples of cotton cloth were: (a) mercerized by treatment with 20% sodium hydroxide; (b) aminoethylated to a D.S. of 0.08 by treatment with 2-aminoethyl sulfuric acid and 40% sodium hydroxide; (c) carbamoylethylated to a D.S. of 0.25 by impregnation with an aqueous solution containing 50% acrylamide and 4% sodium hydroxide followed by heating at 135° C. for five minutes; (d) carboxyethylated to a D.S. of 0.12 by hydrolysis of partially cyanoethylated cotton with 20% sodium hydroxide solution for 16 hours at 25° C.; (e) carboxymethylated to a D.S. of 0.10 by treatment with 17% aqueous chloroacetic acid and 50% sodium hydroxide solution; (f) cyanoethylated to a D.S. of 0.55 by impregnation with 2% sodium hydroxide solution followed by treatment with acrylonitrile at 55° C.; (g) hydroxyethylated to a D.S. of 0.25 by impregnation with 7% sodium hydroxide solution followed by treatment with 10% ethylene oxide in perchloroethylene at 25° C.; (h) phosphonomethylated to a D.S. of 0.04 by treatment with 6.8% disodium salt of chloromethylphosphonic acid in the presence of 25% sodium hydroxide. The fabrics were washed and dried. They were then treated with an aqueous solution containing 70% nitric acid, by weight, for 30 minutes at 26° C. (room temperature), and thoroughly washed with distilled water and dried. The alkali-solubilities of the treated samples are shown in the following table.

Table I

|                                  | Alkali-solubility, Percent |
|----------------------------------|----------------------------|
| Fabric treated with nitric acid: |                            |
| Mercerized cotton                | 65.6                       |
| Aminoethylated cotton            | 97.1                       |
| Carbamoylethylated cotton        | 80.5                       |
| Carboxyethylated cotton          | 100.0                      |
| Carboxymethylated cotton         | 98.3                       |
| Cyanoethylated cotton            | 96.3                       |
| Hydroxyethylated cotton          | 82.7                       |
| Phosphonomethylated cotton       | 82.8                       |

#### EXAMPLE 2

A sample of cotton was hydroxyethylated to a D.S. of 0.50 by treatment similar to that of sample (g) of Example 1. It was treated with nitric acid as in Example 1. The alkali-solubility was 89.5%.

#### EXAMPLE 3

A sample of cotton cloth was phosphonomethylated to a D.S. of 0.09 by treatment similar to that of sample (h) of Example 1. It was treated with nitric acid as in Example 1. The alkali-solubility was 99.3%.

#### EXAMPLE 4

Samples of partially carboxymethylated cotton, D.S. 0.10, were treated with aqueous solutions containing 70%

nitric acid, by weight, at 26° C. for various periods of time of from 5 minutes to 75 minutes. For comparison, a sample of mercerized cotton was treated for 75 minutes. The properties of the treated samples are shown in the following table.

Table II

| Fabric Treated With Nitric Acid | Time of Treatment, Minutes | Alkali Solubility, percent | Strength Retained, percent |
|---------------------------------|----------------------------|----------------------------|----------------------------|
| Carboxymethylated Cotton        | 5                          | 50.2                       | 86.3                       |
| Do                              | 10                         | 87.8                       | 85.0                       |
| Do                              | 15                         | 93.8                       | 76.4                       |
| Do                              | 30                         | 98.3                       | 75.8                       |
| Do                              | 45                         | 98.7                       | 63.3                       |
| Do                              | 60                         | 99.4                       | 67.9                       |
| Do                              | 75                         | 99.4                       | 65.3                       |
| Mercerized Cotton               | 75                         | 73.6                       | 70.7                       |

## EXAMPLE 5

Samples of partially carboxymethylated cotton (D.S. 0.08) and of mercerized cotton cloth were treated with an aqueous solution containing 70% nitric acid, by weight, at 40° C. for 5 minutes. The nitric acid treated-carboxymethylated fabric was 88.4% alkali-soluble and retained 73.5% of its original strength. The nitric acid treated-mercerized fabric was only 53.0% alkali-soluble and retained 89.4% of its original strength.

## EXAMPLE 6

Samples of partially carboxymethylated cotton (D.S. 0.08) and of mercerized cotton were treated with an aqueous solution containing 35% nitric acid, by weight, at the boil for 0.5 minute. Alkali-solubilities were 96.3% and 27.9%, respectively.

## EXAMPLE 7

Samples of partially carboxymethylated cotton (D.S. 0.08) and of mercerized cotton were treated with an aqueous solution containing 10% nitric acid, by weight, at the boil for 4 minutes. Alkali-solubilities were 96.7% and 53.2%, respectively.

We claim:

1. A process for producing an aqueous alkali soluble cotton cellulosic textile material which comprises partially etherifying the cotton cellulosic textile material to a degree of substitution of from about 0.01 to about 0.6 and

oxidizing the cellulose chain of the partially etherified textile material by treating the partially etherified cotton cellulosic textile material with an aqueous solution of nitric acid in a concentration of from about 10% to about 70% by weight, at a temperature of from about room temperature to that of the boiling point of the aqueous nitric acid solution, for a period of time of from about 0.5 minute to about 75 minutes, the time and temperature of the nitric acid treatment being inversely related to the nitric acid concentration.

2. The process of claim 1 in which the partial etherification employed is aminoethylation.
3. The process of claim 1 in which the partial etherification employed is carbamoylethylation.
4. The process of claim 1 in which the partial etherification employed is carboxyethylation.
5. The process of claim 1 in which the partial etherification employed is carboxymethylation.
6. The process of claim 1 in which the partial etherification employed is cyanethylation.
7. The process of claim 1 in which the partial etherification employed is hydroxyethylation.
8. The process of claim 1 in which the partial etherification employed is phosphonomethylation.

## References Cited in the file of this patent

## UNITED STATES PATENTS

2,461,632 Datlow ----- Feb. 15, 1949

## OTHER REFERENCES

Lawrie et al.: J. of the Soc. of Dyers and Colourists, 56 pp. 6-17, 1940.

Guthrie: Textile Research Journal 17, pp. 625-629, 1947.

Frick et al.: Textile Research J. 27, pp. 294-299, 1957.  
Daul et al.: Textile Research J. 25, pp. 246-253, 1955.  
Daul et al.: Textile Research J. 22, pp. 787-792, 1952.  
Daul et al.: Textile Research J. 25, pp. 246-253, 1955.  
Drake et al.: Textile Research J. 29, pp. 270-275, 1959.

Reinhardt et al.: "Industrial and Engineering Chemistry," vol. 50, No. 1, January 1958, pp. 83-86.

Reinhardt et al.: "Textile Research Journal," vol. XXIX, No. 10, October 1959, pp. 802-810, particularly p. 810.